

## UNITED STATES PATENT OFFICE

2,380,838

## MAGNESIUM BASE ALLOY

Joseph D. Hanawalt, Midland, Mich., assignor to  
The Dow Chemical Company, Midland, Mich.,  
a corporation of Michigan

No Drawing. Application November 10, 1941,  
Serial No. 418,615

4 Claims. (Cl. 75—163)

This invention relates to magnesium base alloys and more particularly concerns a magnesium base alloy having desirable physical properties such as excellent formability, yield, and tensile strengths, coupled with a high degree of weldability.

Magnesium alloys are now extensively employed in various structural and mechanical arts where a light weight metal is highly advantageous, such as for use in making castings, forgings, and the like. However, the use of magnesium alloys in rolled form to make sheet metal articles requiring both forming and welding operations has not progressed as rapidly due to the fact that heretofore alloys were not obtainable having a desirable combination of properties, such as excellent formability, tensile and yield strengths, and desirable welding characteristics.

It is, accordingly, the principal object of this invention to provide a magnesium base alloy having excellent formability, high yield and tensile strengths, and a high degree of weldability.

Other objects and advantages of the invention will be apparent as the description proceeds.

My invention resides in the discovery that a magnesium base alloy composed of from 1 to 3 per cent of manganese and from 0.02 to 0.05 per cent of calcium, the balance being substantially all magnesium, possesses the aforementioned properties. The term "magnesium" used herein and in the appended claims is intended to include magnesium containing the ordinary impurities found in the commercially pure metal, such as traces of iron, copper, nickel, and silicon. While the properties of excellent strength, good formability, and desirable welding characteristics are manifest over the entire range of composition indicated, a preferred composition contains from 1.2 to 2 per cent manganese and from 0.03 to 0.04 per cent calcium.

The following table lists some of the properties of rolled sheet made from my new alloy and compares these properties with rolled sheet made from related alloys. A comparison of the properties shows the improvement in strength characteristics, formability, and weldability of my new alloy over that of the closely related alloys. In the table the percent elongation is to be regarded as a measure of the ductility or formability of the specimen.

Table

| 5   | Annealed |    |                                 |                                |                                  |              |
|-----|----------|----|---------------------------------|--------------------------------|----------------------------------|--------------|
|     | Mn       | Ca | Per cent elongation in 2 inches | Yield strength in lbs./sq. in. | Tensile strength in lbs./sq. in. | Weldability. |
| 1.5 | 0        | 4  | 22,000                          | 22,000                         | Excellent.                       |              |
| 1.5 | .03      | 15 | 22,000                          | 22,000                         | Do.                              |              |
| 0   | .05      | 15 | 15,000                          | 31,000                         | Do.                              |              |
| 1.5 | .05      | 17 | 22,000                          | 30,000                         | Do.                              |              |
| 1.5 | .07      | 18 | 22,000                          | 35,000                         | Poor.                            |              |
| 1.5 | .09      | 18 | 22,000                          | 35,000                         | Very poor.                       |              |
| 1.5 | .12      | 19 | 22,000                          | 35,000                         | Do.                              |              |

The properties listed in the above table under the section headed "Annealed" were obtained by first rolling the alloys at a temperature of 500° to 700° F. and thereafter annealing them at a temperature of 600° to 700° F. A comparison of the properties listed in the table shows that the combined properties of the new alloy are greatly superior to those of the related alloys having similar percentages of alloying ingredients. Thus, it will be noted that the new alloy containing both manganese and calcium showed a high degree of improvement in its combined properties over that of the binary magnesium-manganese alloy or the binary magnesium-calcium alloy.

It has been found that it is essential to have at least 0.02 per cent of calcium present in the alloy composition in order to obtain a high degree of elongation and thus excellent formability characteristics. At the same time, it has been found that the per cent of calcium present in the alloying composition must not exceed about 0.05 or sheets made from the alloy do not possess good welding characteristics. For example, if the calcium content of the alloy exceeds about 0.05 per cent, cracks develop in and about the weld bead rendering the weld unsatisfactory. This cracking tendency is especially noticeable if the weld is stressed to any degree. However, a composition containing between about 0.02 and 0.05 per cent of calcium possesses excellent formability characteristics as shown by the table, and, at the same time, the composition is suitable for use where welds are to be made. The new alloy

is, of course, most useful in the form of sheets and the like wherein a welding operation is necessary to complete the fabrication of the finished article such as in making airplane tanks from sections of magnesium sheet, although it may also be suitably used in making castings, forgings, extruded forms and the like.

It is further pointed out that my new alloy is amenable to solution and precipitation heat treatments which, accordingly, modify its properties.

The new alloy may be prepared by any of the methods employed for melting and alloying materials with magnesium, such as by adding the respective materials singly or jointly to a bath of molten magnesium which is preferably protected from oxidation by a suitable flux.

I claim:

1. A magnesium base alloy containing from 1.3 to 2 percent of manganese and from 0.03 to 0.04 per cent of calcium, the balance being substantially all magnesium.

2. A magnesium base alloy containing 1.5 per cent of manganese and 0.04 per cent of calcium, the remainder being substantially all magnesium.

3. A welded article containing from 1 to 3 per cent of manganese, 0.02 to 0.05 per cent of calcium, the remainder being substantially all magnesium.

4. A magnesium base alloy containing from 1 to 3 per cent of manganese and from 0.02 to 0.05 per cent of calcium, the balance being substantially all magnesium.

JOSEPH D. HANAWALT.